

April 15, 1924

1,490,450

C. W. BROKATE

PROTECTED DRY CELL BOBBIN AND METHOD OF MAKING THE SAME

Filed Feb. 26, 1921



Inventor:

*Charles W. Brokate,  
J. Byers, Townsend & Bickerton,*

Attorneys.

Patented Apr. 15, 1924.

1,490,450

# UNITED STATES PATENT OFFICE.

CLARENCE W. BROKATE, OF FREMONT, OHIO, ASSIGNOR TO NATIONAL CARBON CO. INC., A CORPORATION OF NEW YORK.

## PROTECTED DRY-CELL BOBBIN AND METHOD OF MAKING THE SAME.

Application filed February 26, 1921. Serial No. 448,241.

To all whom it may concern:

Be it known that I, CLARENCE W. BROKATE, a citizen of the United States, residing at Fremont, in the county of Sandusky and 5 State of Ohio, have invented certain new and useful Improvements in Protected Dry-Cell Bobbins and Methods of Making the Same, of which the following is a specification.

10 This invention relates to improvements in that type of dry cells in which the cathode is a carbon rod carrying a molded mix bobbin or core. In cells of this kind the bobbin is usually enclosed in a wrapper of gauze, 15 cheese cloth or like fabric, suitably tied in position. The object of my invention is to eliminate the tedious and expensive operations of wrapping and tying, by the substitution for the fabric of a more efficient and 20 economical protective means.

Molded mix bobbins are relatively fragile. They are likely to be injured by handling before insertion in the cells, and when inserted they may scale or crumble due to the 25 softening action of the electrolyte or for other reasons. As no isolating lining for the active surface of the zinc electrode is usually provided in cells having the mix in molded form, the crumbling of the bobbin is 30 a serious disadvantage and must be prevented. Particles of carbonaceous material and manganese dioxid may be dislodged when the bobbin is inserted or may work their way or migrate through the paste of excit- 35 ant and come into contact with the zinc, setting up wasteful local action with perforation of the zinc and leakage of electrolyte. To prevent these and other troubles the wrapping method referred to is now com- 40 monly used.

I have discovered that by proceeding as hereinafter fully set forth I obtain a protective bobbin coating which performs all the useful functions of the gauze wrapping 45 and is economical and easily applied. Broadly, the method consists in precipitating a chemical compound at or near the exterior surface of the bobbin.

In the accompanying drawing illustrative 50 of the invention, the figure is a vertical central section through a dry cell. In this drawing, reference numeral 1 denotes a depolarizing core or bobbin formed about a carbon rod 2 and inserted in a metal elec- 55 trode 3 containing excitant 4. The protec-

tive coating 5, hereinafter described in detail, overlies the bobbin surface and permeates the outer portion of the mix, securely bonding the same. The bobbin may rest on a spacing disc 6. A seal 7 closes the cell. 60

In the preferred embodiment of my invention, bobbins containing a salt of an alkaline earth metal, e. g. calcium or barium chlorid, are brought into contact with a solution of a soluble sulfate, for example, ammonium sulfate or zinc sulfate. By the resulting double decomposition an insoluble superficial layer of calcium or barium sulfate is formed upon the bobbin. This layer of precipitated salt acts as a cement or binder, unifying and strengthening the exposed surface of the mix. Bobbins so protected may be safely handled and do not disintegrate in use. 70

Alkaline earth metal chlorid in quantity 75 in excess of that required to produce the coating is preferably incorporated with the mix ingredients before molding. For example, a mix comprising manganese dioxid and carbon or graphite may be moistened 80 with the usual electrolyte of zinc chlorid and ammonium chlorid, to which has been added the proper amount of alkaline earth metal chlorid. The quantity of the chlorid may be varied within wide limits but I prefer to 85 use it in the proportion of approximately 6 parts by weight of dry chlorid to 100 parts of mix. The moistened materials are then molded about a carbon rod, and the bobbin so formed is immersed in a solution of a sulfate, forming the cementing precipitate. The cell may be completed in the usual way 90 by inserting the protected bobbin axially in a zinc container, applying excitant paste between the bobbin and container, and sealing 95 in the customary manner.

The thickness of the protective layer may of course be regulated by varying the concentration of the reacting solutions and the time of immersion in the precipitant. In 100 general, a superficial coating only is required. By examining a treated bobbin the depth to which precipitation has extended may be readily determined and the concentration and time of reaction adjusted to obtain a greater or less depth as desired. The character of the coating will depend somewhat upon the nature of the mix materials. I have found that a firmer, smoother coating may be obtained if the carbonaceous mate- 110

rial and depolarizer are very finely divided, and I prefer to pass these materials through at least a hundred-mesh screen.

Instead of incorporating the alkaline earth metal chlorid with the electrolyte before molding, the bobbin in molded form may be dipped into a solution of the chlorid and then treated with a soluble sulfate. This necessitates two immersing operations instead of one and in general all the alkaline earth metal chlorid, being adjacent to the surface impregnated by the sulfate, will react with it. The presence of alkaline earth metal chlorids in the dry cell mix is advantageous, tending to prevent gassing, as has been shown in the patent application of Anna F. MacKenzie, Ser. No. 412,744, filed November 4, 1920. For this reason I prefer to disseminate the chlorid throughout the entire mass of the bobbin using an excess as described above.

While the metathesis of two salts is probably the most convenient way of obtaining the cementing precipitate, it is evident that other types of reaction may be employed. For example, an alkaline earth metal oxid or hydroxid may be caused to react at the surface of the bobbin with a soluble sulfate or sulfuric acid. In any case the treated bobbin may be washed or neutralized, though this will not in general be necessary.

The invention is not limited to the formation of insoluble sulfates upon the bobbin surface, as many other precipitations in situ will have a satisfactory binding action. For example, I have used phosphates in this connection with advantage.

From the foregoing description it will be clear that the making of a protected bobbin according to my invention involves only processes which can be carried out mechanically and simultaneously upon a large number of elements. It has been found in practice that bobbins thus indurated by precipitation are self-sustaining and free from tendency to crumble. Also, the in-

soluble coating does not appreciably increase the internal resistance of the cell nor diminish the porosity of the mix, and the coating volume is relatively so small that the capacity of the cell for holding active material is practically undiminished.

In the appended claims, the qualification "insoluble" is used for brevity in designating substances which have a negligible solubility in water or the electrolyte of dry cells.

I claim:

1. In a process of making a protected bobbin, applying to the bobbin a solution containing a precipitable material, and then reacting upon the solution with a precipitant for such material.

2. In a process of making a protected bobbin chemically, precipitating an insoluble sulfate upon and beneath the surface of the bobbin.

3. In a process of making a protected bobbin, precipitating barium sulfate upon and beneath the surface of the bobbin.

4. In a process of making a protected bobbin, adding to the usual bobbin constituents an additional substance, and applying a material adapted to form a precipitate with said substance.

5. In a process of making a protected bobbin, incorporating with the usual bobbin constituents an additional substance, molding a bobbin containing said constituents and substance, and applying to the molded bobbin a material adapted to form a precipitate with said substance.

6. In a process of making a protected bobbin, incorporating an alkaline earth metal chlorid with the usual bobbin constituents, molding a bobbin therefrom, and applying a soluble sulfate to the molded bobbin.

7. A dry cell bobbin provided with a coating of barium sulfate.

In testimony whereof I affix my signature.

CLARENCE W. BROKATE.